

# UNITED STATES PATENT OFFICE.

THOMAS A. JANNEY, OF GARFIELD, AND CHARLES M. NOOKES, OF SALT LAKE CITY,  
UTAH.

## PROCESS OF CONCENTRATING ORES.

1,281,018.

Specification of Letters Patent.

Patented Oct. 8, 1918.

No Drawing.

Application filed July 28, 1917. Serial No. 183,316.

*To all whom it may concern:*

Be it known that we, THOMAS A. JANNEY, a citizen of the United States, residing at Garfield, in the county of Salt Lake and 5 State of Utah, and CHARLES M. NOOKES, a citizen of the United States, residing at Salt Lake City, in the county of Salt Lake and State of Utah, have invented certain new and useful Improvements in Processes of 10 Concentrating Ores, of which the following is a specification.

The object of this invention is to provide more economical means for the concentration of ores by the flotation process, and to 15 combine with such economy greater effectiveness in point of the amount of metal recovered and the purity of the concentrate.

Our improved process effects the desired economy by reason of the fact that we are 20 able to use oils which are very abundant and cheap, rendering these oils effective to produce the desired result by dissolving therein a proportion of gilsonite. In some instances we have found it advisable to add 25 to the mixture a third ingredient consisting of some frothing oil, this, however, not being necessary in all cases. There are a large number of oils which are efficient agents for the production of froth or bubbles, but 30 which in themselves lack the property of effecting an efficient separation of the metalliferous mineral from the gangue. Some oils are effective to produce bubbles or froth, and in connection with some ores also bring 35 about the separation of metalliferous mineral from gangue, but the same oils when applied to other ores while effective to cause the formation of bubbles or froth, fail to bring about an efficient separation of the 40 metalliferous mineral from the gangue. For instance, pine oil, when used in connection with the slimes of the Utah copper ore, either with or without mineral acid, will produce an abundance of bubbles or froth, 45 but no efficient separation of the metalliferous mineral from the gangue. If pine oil, however, be used in connection with the solution of gilsonite in crude petroleum or petroleum distillate, the slimes of the Utah 50 copper ore may be concentrated with the highest degree of efficiency, both as to the recovery and grade of concentrate.

While the solution of gilsonite in petroleum or a petroleum distillate and in some 55 cases, with some bubble forming substance

added is an efficient flotation agent, it has been found that neither of the oils mentioned, when taken alone, is effective to produce an efficient result in connection with many ores, and in connection with other 60 ores, the result produced by pine oil or petroleum alone is less efficient than that produced by the mixture named. The application of a low degree of heat hastens the solution of the gilsonite in the petroleum, 65 but without the application of heat, the gilsonite will dissolve, but more slowly.

Gilsonite may be used to advantage with other oils and oily substances than the petroleum products, but we have mentioned crude 70 petroleum and petroleum distillate by reason of the fact that they are cheap and serve the purpose efficiently.

The mixture of gilsonite with petroleum, or other oily substance, and some substance 75 like pine oil, which has the property of producing bubbles or froth, is not restricted to any particular method of carrying out the flotation process. The process may be carried out by the method of beating air into 80 the pulp by mechanical agitation, with the result of producing a coherent and permanent froth, or the agitation may be dispensed with and the air may be introduced through a porous medium forming part of the vessel 85 containing the pulp, thus giving rise to the formation of evanescent bubbles which must be quickly collected, or gases other than air produced chemically or electrolytically may be utilized. 90

As an example of our process, we have used in connection with the slimes of the Utah Copper Company's ore a mixture consisting of 40% of gilsonite and 60% of kerosene distillate. We have also used a mixture consisting of 90% California fuel oil and 10% of gilsonite in solution. We have also used various other petroleum distillates with varying amounts of gilsonite in solution. In treating the slimes of the Utah 100 copper ore, we have added the petroleum-gilsonite solution in the proportion of 20 lbs. per ton of solids contained in the pulp, and have added thereto pine oil in the proportion of about one pound per ton of solids 105 in the pulp. In using this mixture, we used about five pounds of sulfuric acid per ton of material treated. The pulp with the re-agents named was first stirred sufficiently to distribute the re-agents throughout the 110

pulp. After the pulp and re-agents were mixed, the pulp was conducted to a cell provided with a porous wall through which air was caused to percolate into the pulp. The 5 air bubbles rising through the pulp collected the metalliferous mineral and were removed from the surface in the form of a concentrate of higher grade and effecting a greater recovery than had been accomplished by 10 methods heretofore in use.

The operation above described was in one instance conducted for a period of eight hours, during which time about 260 tons of material were treated. The average results 15 for 8 hours were as follows: Heads—1.03% copper; Tailings—.08% copper; Concentrate—19.9% copper, 19% iron, and 26% silica.

The extraction indicated by the figures 20 above was 92.61%. On other occasions the silica contained in the concentrate, operating under similar conditions, was much less.

Acid, alkalis, salts, or other re-agents may be used in connection with the gilsonite 25 mixture when the treatment of any particular ore is improved by the use of said re-agents, and the temperature and other factors may be adjusted to obtain the best results as is usual in the use of other oils and 30 oil mixtures.

What we claim is:

1. A process of concentrating ores consisting in forming a mixture of the ground 35 ore with water, adding thereto a solution of gilsonite in oil, and aerating the pulp.

2. A process of concentrating ores consisting in forming a mixture of the ground ore with water, adding thereto a solution of

gilsonite in oil, adding another oil having greater frothing power than said first named 40 oil, and aerating the pulp.

3. A process of concentrating ores consisting in forming a mixture of the ground ore with water, adding thereto a solution of gilsonite in oil, adding another oil having 45 greater frothing power than said first named oil, adding a suitable acid re-agent to the pulp, and aerating the pulp.

4. A process of concentrating ores consisting of forming a mixture of the ground 50 ore with water, adding thereto a solution of gilsonite in oil, adding another oil having greater frothing power than said first named oil, adding a suitable reagent to the pulp, and aerating the pulp.

5. A process of concentrating ores consisting in forming a mixture of ground ore with water, oil having a mineral selective action, oil having a frothing action, and gilsonite, and aerating the resultant mixture 60 to concentrate the metalliferous content thereof.

6. A process of concentrating ores consisting in forming a mixture of ground ore with water, oil having a mineral selective 65 action, oil having a frothing action, gilsonite, and a suitable quantity of a re-agent, and aerating the resultant mixture to concentrate the metalliferous content thereof.

In testimony whereof we have subscribed 70 our names.

THOMAS A. JANNEY,  
CHAS. M. NOKES.

Witnesses:

C. Y. PFOUTZ,  
A. C. FRENCH